

# UNITED STATES PATENT OFFICE.

ANGELO LUCERTINI, OF SAMPIERDARENA, ITALY, ASSIGNOR TO SOCIETÀ ANONIMA ITALIANA GIO. ANSALDO ARMSTRONG & CO., OF GENOA, ITALY.

## PROCESS FOR THE MANUFACTURE OF ARMOR-PLATES.

1,086,459.

Specification of Letters Patent.

Patented Feb. 10, 1914.

No Drawing.

Application filed April 20, 1912. Serial No. 692,144.

To all whom it may concern:

Be it known that I, ANGELO LUCERTINI, a subject of the King of Italy, and residing at No. 69 Via Cristoforo Colombo, Sampierdarena, Italy, have invented a certain new and useful Process for the Manufacture of Armor-Plates, of which the following is a specification.

This invention relates to an improved process for the manufacture of armor plates for naval and the like purposes based on the employment of a metal which has not yet been used for cemented armor plates. According to this invention this metal having been previously rolled and forged is subjected to a first series of thermal treatments, then to a short cementation process and finally to a second series of thermal treatments.

10 The improved process is carried out as follows:—

1. Manufacture of an ingot of Martin steel having approximately the following chemical composition:—Carbon 0.50 to 0.70, silicon 0.100 to 0.150, sulfur and phosphorus < 0.035, manganese 0.25 to 0.40, chromium 1.80 to 2.50, nickel 3.50 to 4.50.

The principal operation in the manufacture of steel which must always be borne in mind, is the regulation of the temperature of the bath of molten metal by maintaining it at as low a degree as possible while yet sufficient to allow and insure the complete fusion of the final additions so that the metal can be run readily into the ingot molds. Any excess of temperature beyond what is absolutely necessary for satisfying those requirements is to be considered as injurious to the mechanical properties of the metal.

2. The steel ingot taken from the ingot mold is placed in a furnace and maintained therein at a constant temperature of about 450 degrees C. for a long period of several hours, said period varying with the dimensions of the ingots. The length of time during which the ingots remain in the furnace at a low temperature, varies in direct ratio with the weight of the ingots, commencing with a minimum of 25 hours for small armor plate ingots of about 12 tons weight each. The said length of time is to be taken as a minimum for ingots of almost round or rectangular form instead of the flat or plate form usually adopted for armor plates.

3. The ingot is then placed in a furnace wherein it is heated for rolling or forging, the heating being effected gradually until a uniform temperature of about 1200 degrees C. is reached.

4. The rolling or forging is effected preferably with the aid of repeated annealings and successive lowerings of the temperature of the whole plate down to about 400 degrees C., carried out in a stove or even in the midst of a mass of ashes.

5. The armor plate is now subjected to the following series of thermal treatments:—Heating to a temperature of about 600 degrees C., and quenching in oil or lukewarm water. Then heating to a temperature of from about 750 to 780 degrees C., and upsetting of the armor plate, care being taken, especially during this heating to eliminate by means of the press the most pronounced bends due to the rolling or forging operation, and which it is too risky to eliminate by heating to a low temperature. The armor plate thus upset is allowed to cool down to a uniform temperature of about 200 degrees C., in oil or even in a tank of boiling water. It is then immediately placed in the furnace, heated with care to a uniform temperature of about 630 degrees C., and carefully upset, after which the armor plate is allowed to cool freely in the air. It is preferred to subject it to the mechanical operation of planing on its face which is intended to be cemented. Although this planing is not absolutely necessary, it is however suitable for the purpose of removing the roughness and any other superficial faults that may become apparent after the rolling or forging operation.

6. The armor plate is now subjected to the cementing operation which is effected by the use of cementing gases produced by special generating devices, or by the use of mixtures of animal or vegetable charcoal, or by any other method, in a very short time, by keeping the plate in contact with the cementing agent during a period of about 60 hours at a temperature of from 960 to 1000 degrees C. This short period is sufficient to raise the face of the plate by a superficial percentage of 1 per cent. of carbon.

In view of the exceptional shortness of the cementation period, the most suitable method which corresponds by its efficiency to the thermal requirements is the method

which is based on the use of carbonic oxide because this method has the great advantage of producing cementation to a depth which can be predetermined and of constant intensity at all points thereof.

- 5 On the termination of the cementation period the temperature is allowed to fall to about 780-800 degrees C., and the plate is immersed in oil until it has cooled down further to about 300-400 degrees C. The armor plate is then placed in the furnace wherein it is heated gradually and uniformly to a temperature of 625-640 degrees C., whereupon it is quenched in water.
- 10 15 The armor plate is then subjected to a second series of thermal treatments as follows:—The armor plate is heated to a temperature of 750-780 degrees C., this temperature being utilized for bending the armor plate into its final form. As soon as this is completed, the plate, whatever its temperature may now be, is then placed immediately again into the furnace, heated to a temperature of 750-780 degrees C., and again 20 25 quenched in oil. The plate is removed from the oil while still hot, and it is immediately put back into the furnace wherein it is heated with care to a temperature of about 635 degrees C. It is then quenched in water.
- 30 35 After this operation the armor plate is machined to the desired shape after having first taken a sample from it by means of a chisel for breaking in the press for the purpose of examining the structure of the metal. The armor plate is at the same time prepared 40 45 for subjection to the final treatment of differential hardening, portions being left at the ends as usual for the successive examination of its appearance after this operation.
- 45 50 Before proceeding to the final hardening, the appearance of the fracture after the last quenching at 635 degrees C., is noted. If the fracture has a fibrous or approximately fibrous appearance, the final hardening is then proceeded with. If however the fracture has a pearly or granular appearance the quenching in water at 635 degrees C., must be repeated. Finally the differential hardening is effected with the greatest care, 55 60 the face of the plate being heated to a temperature of 850 degrees C., and its back which is in contact with a bed of sand being heated to a temperature of about 600 degrees C. The plate is then quenched.

55 What I claim is:—

1. The process of making armor plate comprising the following steps: subjecting the plate to repeated temperings, cementing the plate, repeatedly tempering the cemented plate, heating the face of the plate above the recalcene point, while maintaining the back at a lower temperature, then quenching the plate.
- 60 65 2. The process of making armor plate comprising the following steps: annealing

the steel ingot and after forging subjecting the plate to repeated temperings, cementing the plate, repeatedly tempering the cemented plate, heating the face of the plate above the recalcene point, while maintaining the back at a lower temperature, then quenching the plate.

3. The process of making armor plate comprising the following steps: heating a plate to 600° C. and quenching in water at 75 100° C., reheating to 750°, cooling to 200° by quenching, cementing the plate, heating the cemented plate to 750° C., quenching; reheating to 635° C. and quenching; heating the face of the plate above the recalcene 80 point while maintaining the back at a lower temperature, then quenching the plate.

4. The process of making armor plate comprising the following steps: annealing the steel ingot and after forging subjecting 85 the plate to repeated temperings, cementing the plate, repeatedly tempering the cemented plate, then heating the face of the plate to 850° C. while maintaining the back at a temperature not exceeding 600°, then quenching 90 the plate.

5. The process of making armor plate comprising the following steps: annealing the steel ingot and after forging subjecting the plate to repeated temperings, cementing 95 the plate for 60 hours at a temperature of 960 to 1000° C., repeatedly tempering the cemented plate, heating the face of the plate above the recalcene point, while maintaining the back at a lower temperature, 100 then quenching the plate.

6. The process of making armor plate comprising the following steps: annealing the steel ingot and after forging, heating the plate to 600° C. and quenching in water at 105 100° C.; reheating to 750° cooling to 200° by quenching; again heating to 630° for bending, cementing the plate; heating the cemented plate to 750°, quenching; reheating to 635° C. and quenching; heating the face 110 of the plate above the recalcene point while maintaining the back at a lower temperature, then quenching the plate.

7. The process of making armor plate comprising the following steps: annealing 115 the steel ingot and after forging, heating the plate to 600° C. and quenching in water at 100° C.; reheating to 750° cooling to 200° by quenching, again heating to 630° for bending; cementing the plate; heating the cemented plate to 750°, quenching; reheating to 635° C. and quenching; heating the face of the plate to 850° while maintaining the back at 600°, then quenching the plate.

8. The process of making armor plate 125 comprising the following steps: heating the plate to 600° C. and quenching in water at 100° C.; reheating to 750° cooling to 200° by quenching, again heating to 630° for bending; cementing the plate for 60 hours in con- 120

tact with carbon at a temperature of 960-1000°; heating the cemented plate to 750°, quenching, reheating to 635° C. and quenching; heating the face of the plate to 850° while maintaining the back at 600°, then quenching the plate.

9. The process of making armor plate comprising the following steps: annealing the steel ingot and after forging, heating the plate to 600° C. and quenching in water at 100° C.; reheating to 750°, cooling to 200° by quenching, again heating to 630° for bending; cementing the plate for 60 hours in

contact with carbon at a temperature of 960-1000°; heating the cemented plate to 750°, 15 quenching, reheating to 635° C. and quenching; heating the face of the plate to 850° while maintaining the back at 600°, then quenching the plate.

In testimony whereof I have signed my 20 name to this specification in the presence of two subscribing witnesses.

ANGELO LUCERTINI.

Witnesses:

DUILIO NARVONI,  
NICOLA SISTO.